

# UNITED STATES PATENT OFFICE.

JULIUS ALEXANDER, OF ALTONA, GERMANY.

## BRIQUET.

1,117,125.

Specification of Letters Patent. Patented Nov. 10, 1914.

No Drawing.

Application filed December 3, 1913. Serial No. 804,406.

To all whom it may concern:

Be it known that I, JULIUS ALEXANDER, a subject of the German Emperor, and a resident of 11 Ottensen Marktplatz, Altona, 5 Germany, have invented certain new and useful Improvements in Briquets, of which the following is a statement.

In the working of railways combustible waste products are obtained in form of coke 10 dust (cinders from the smoke box of the engines), saw dust and wood shavings, and other combustible waste products such as oil gas tar and lamp black are obtained in the production of oil gas. Of these waste 15 products sawdust and coke dust have been employed in the production of briquets, but these materials could not be used with the customary methods employing pitch or coal tar or other viscous tars resulting in 20 the dry distillation of solid raw materials as binding medium, as, even under high pressure, the pitch or tar will bind the particles of coke or saw dust together on their surface only, whereas the air contained in 25 the numerous pores is firmly inclosed in the compression and cannot escape. The result of this is that such briquets, when they are fired on the grate, quickly fall to pieces, as experience has shown, as the air contained 30 in the pores expands already at the commencement of the combustion and thereby cause the briquets to fall to pieces even before any intensive combustion could take place. Thereby the whole object of briquetting the coke or sawdust which in the 35 non-briquetted condition can only be burnt on special grates with under-grate blast entailing high working expenses is nullified. Even crude petroleum which has been also 40 suggested as a binding medium, cannot fulfil its purpose, because its binding power is extremely small and necessitates considerable pressure for the compression which essentially increases the cost of production of the 45 briquets.

According to the present invention a binding medium is used for briquetting coke dust and the like which binding medium, serving as substitute for the aforementioned pitch

or coal tar consists of a thin liquid tar obtained in the manufacture of oil gas, which, as has been shown by experiments, is capable of entering into the pores of the coke and driving out the air therein contained already at a pressure of 100 atmospheres. 50 At the same time this tar constitutes a much better binding medium as compared with the coal tar hitherto used as such, because in the normal conversion of gas oils into gas about 30% of the same pass over partly 55 unchanged and partly in form of liquid and thick hydrocarbons into the precipitated oil gas tar and considerably increase, as compared to coal tar, the binding efficiency of the same and its calorific value (about 10600 60 heat units). These advantages of the oil gas tar as a binding medium are still further increased according to the present invention by the fat or oil soot depositing in 65 the retorts and pipes being added to it. 70

According to the present invention, thus, a high-value briquet is produced of a calorific value of about 6900 heat units, which, as careful tests have shown, can already be produced at a pressure of 100 atmospheres, 75 and which, when burnt on an ordinary grate will retain its coherence like ordinary mineral coal.

The components mentioned hereinbefore are preferably mixed at the following ratio: 80 9 parts of wood waste; 85 parts of coke cinders or coke dust; 6 parts of oil gas tar. In place of the latter 6 parts of oil gas tar also equal parts of oil gas tar and oil soot may be used thus giving the following formula: 9 parts of wood waste; 85 parts of coke cinders or coke dust; 3 parts of oil gas tar; 3 parts of oil soot. This mixture is then pressed under an ordinary briquetting press at a pressure of 100 atmospheres into 85 the form of briquets. It has, however, been found that the briquets may be made after the present method also of coke dust or fine coke alone without any addition of wood waste. 90

I claim:

A composition for briquets consisting of coke dust, wood waste, and a binding mate-

rial comprising oil gas tar, and oil soot, the several ingredients being mixed together in about the proportions specified and compressed into briquets, the finished briquets retaining the volatile matter of the binding material.

In testimony whereof I have hereunto

affixed my signature in the presence of two subscribing witnesses.

JULIUS ALEXANDER.

Witnesses:

ERNEST H. L. MUMMENHOFF,  
IDA CHRIST. HAERMAN.

---

Copies of this patent may be obtained for five cents each, by addressing the "Commissioner of Patents, Washington, D. C."